# EUROPEAN PATENT APPLICATION

(11) **EP 4 786 669 A1**
(43) Date of publication of application: **05.08.2026**
(21) Application number: 24872185.4
(22) Date of filing: 24.09.2024
(51) Int. Cl.: D04H 3/011, D04H 3/037, D04H 3/16

(54) **THREE-DIMENSIONAL MESH-LIKE STRUCTURE**

(30) Priority: 27.09.2023 JP 2023165925
(71) Applicant: TOYOBO MC Corporation, Osaka-shi, Osaka 530-0001 (JP)
(72) Inventor: KAWANO, Fumika, Otsu-shi, Shiga 520-0292 (JP); TANIGUCHI, Keisuke, Otsu-shi, Shiga 520-0292 (JP); HENMI, Tatsuya, Otsu-shi, Shiga 520-0292 (JP)
(74) Representative: Müller-Boré & Partner Patentanwälte PartG mbB
(86) International application number: PCT/JP2024/033944
(87) International publication number: WO 2025/070395

(57) **Abstract**

It is provided that a biodegradable three-dimensional network structure that has excellent repeated compression characteristics and excellent compression recoverability after thermal compression at a usage environment temperature. A three-dimensional network structure having a three-dimensional random loop-bonded configuration and comprising a continuous filament made from a thermoplastic resin composition, wherein the thermoplastic resin composition contains 70% by mass or more of a polybutylene adipate terephthalate resin, an enthalpy of an endothermic peak, in which a differential scanning calorimetry curve regarding the continuous filament measured by using a differential scanning calorimeter has a minimum value in a range from 30°C to 70°C, is 2.5 J/g or less, the continuous filament has an average fiber diameter of 0.1 mm or more and 3.0 mm or less, an average fiber diameter of a surface layer portion of the three-dimensional network structure is not less than 1.05 times an average fiber diameter of an inner layer portion of the three-dimensional network structure, and the three-dimensional network structure has an apparent density of 0.01 g/cm³ or more and 0.20 g/cm³ or less, a residual strain after 750-N constant load repeated compression of 15% or less, and a 40%-compression hardness retention rate after 750-N constant load repeated compression of 45% or more.

## Description

### TECHNICAL FIELD

The present invention relates to a three-dimensional network structure.

### BACKGROUND ART

To date, three-dimensional network structures are widely used as cushioning materials utilized for furniture, beddings such as beds, seats for vehicles such as electric trains, automobiles, and two-wheeled vehicles from the viewpoint of excellent air permeability and recyclability. Environment-related issues have been addressed in an accelerated manner recently. In view of this acceleration, research on biodegradable polymers that degrade in a shorter time than conventional polymers has been progressing for these three-dimensional network structures as well. Consequently, various technologies regarding biodegradable three-dimensional network structures have been disclosed to date.

Patent Document 1 discloses a technology of improving plant retaining properties of a biodegradable network structure. In addition, Patent Document 2 discloses a technology of improving local joining of a fiber material of a biodegradable network structure. In addition, Patent Document 3 discloses a technology of forming a coil spring-shaped or loop-shaped portion in a biodegradable three-dimensional structure so as to allow the portion to be suitably deformed under a compressive stress so that the stress is dispersed.

### CITATION LIST

### PATENT DOCUMENT

Patent Document 1: Japanese Laid-Open Patent Publication No. 2001-032236
Patent Document 2: Japanese Laid-Open Patent Publication No. 2020-128608
Patent Document 3: Japanese Laid-Open Patent Publication No. 2000-328422

### SUMMARY OF THE INVENTION

### PROBLEMS TO BE SOLVED BY THE INVENTION

In this manner, various attempts have been made to improve functions of biodegradable network structures to date. However, there has yet to be a known biodegradable three-dimensional network structure that has excellent cushioning properties and that has excellent repeated compression characteristics and excellent recoverability under heating compression at a usage environment temperature at which the three-dimensional network structure is used as a cushioning material. The present invention has been made in view of the above circumstances, and an object of the present invention is to provide a biodegradable three-dimensional network structure that has excellent repeated compression characteristics and excellent compression recoverability after thermal compression at a usage environment temperature. The phrase "has excellent repeated compression characteristics" means that, even after the three-dimensional network structure is repeatedly compressed, the characteristics thereof do not become significantly inferior to those before the repeated compression.

### SOLUTION TO THE PROBLEMS

That is, the present invention has the following invention.
[1] A three-dimensional network structure having a three-dimensional random loop-bonded configuration and comprising a continuous filament made from a thermoplastic resin composition, wherein the thermoplastic resin composition contains 70% by mass or more of a polybutylene adipate terephthalate resin, an enthalpy of an endothermic peak, in which a differential scanning calorimetry curve regarding the continuous filament measured by using a differential scanning calorimeter has a minimum value in a range from 30°C to 70°C, is 2.5 J/g or less, the continuous filament has an average fiber diameter of 0.1 mm or more and 3.0 mm or less, an average fiber diameter of a surface layer portion of the three-dimensional network structure is not less than 1.05 times an average fiber diameter of an inner layer portion of the three-dimensional network structure, and the three-dimensional network structure has an apparent density of 0.01 g/cm³ or more and 0.20 g/cm³ or less, a residual strain after 750-N constant load repeated compression of 15% or less, and a 40%-compression hardness retention rate after 750-N constant load repeated compression of 45% or more.
[2] The three-dimensional network structure according to the above [1], wherein the polybutylene adipate terephthalate resin contains an adipic acid residue and a terephthalic acid residue, and a molar ratio of the terephthalic acid residue to the adipic acid residue is 1.0 or more and 3.0 or less.
[3] The three-dimensional network structure according to the above [1] or [2], wherein the polybutylene adipate terephthalate resin has a melting point of 125°C or more and 180°C or less.
[4] The three-dimensional network structure according to any one of the above [1] to [3], wherein the three-dimensional network structure has a 65%-compression hardness retention rate after 750-N constant load repeated compression of 60% or more.
[5] The three-dimensional network structure according to any one of the above [1] to [4], wherein the three-dimensional network structure has a compressive deflection coefficient of 2.5 or more.
[6] The three-dimensional network structure according to any one of the above [1] to [5], wherein the three-dimensional network structure has a thickness of 10 mm or more and 300 mm or less.
[7] The three-dimensional network structure according to any one of the above [1] to [6], wherein the three-dimensional network structure has a 40°C-compression residual strain of 25% or less.

### EFFECTS OF THE INVENTION

According to the present invention, the above configuration makes it possible to provide a biodegradable three-dimensional network structure that has excellent repeated compression characteristics and excellent compression recoverability after thermal compression at a usage environment temperature.

### BRIEF DESCRIPTION OF THE DRAWING

[FIG. 1] FIG. 1 shows an example of a differential scanning calorimetry curve regarding a continuous filament composing a three-dimensional network structure, the differential scanning calorimetry curve being for measuring an enthalpy of an endothermic peak in which the differential scanning calorimetry curve has a minimum value in a range from 30°C to 70°C.

### DESCRIPTION OF EMBODIMENTS

The three-dimensional network structure of the present invention is a three-dimensional network structure having a three-dimensional random loop-bonded configuration and comprising a continuous filament made from a thermoplastic resin composition, wherein the thermoplastic resin composition contains 70% by mass or more of a polybutylene adipate terephthalate resin, an enthalpy of an endothermic peak, in which a differential scanning calorimetry curve (DSC curve) regarding the continuous filament measured by using a differential scanning calorimeter has a minimum value in a range from 30°C to 70°C, is 2.5 J/g or less, the continuous filament has an average fiber diameter of 0.1 mm or more and 3.0 mm or less, an average fiber diameter of a surface layer portion of the three-dimensional network structure is not less than 1.05 times an average fiber diameter of an inner layer portion of the three-dimensional network structure, and the three-dimensional network structure has an apparent density of 0.01 g/cm³ or more and 0.20 g/cm³ or less, a residual strain after 750-N constant load repeated compression of 15% or less, and a 40%-compression hardness retention rate after 750-N constant load repeated compression of 45% or more.

The above configuration enables improvement of the repeated compression characteristics and the compression recoverability after thermal compression at a usage environment temperature. The usage environment temperature means a temperature at which the three-dimensional network structure of the present invention is used as a product such as a cushion. In the present invention, the usage environment temperature is 40°C. In other words, a 40°C-compression residual strain is regarded as an index of the compression recoverability after thermal compression at the usage environment temperature.

Hereinafter, each of the configurations will be described in detail.

### <Thermoplastic Resin Composition>

The thermoplastic resin composition forming the continuous filament contains 70% by mass or more of a polybutylene adipate terephthalate resin. By selecting the polybutylene adipate terephthalate resin from among biodegradable resins and using the thermoplastic resin composition containing 70% by mass or more of the polybutylene adipate terephthalate resin, a biodegradable three-dimensional network structure having excellent cushioning properties can be obtained. The polybutylene adipate terephthalate resin content is preferably 75% by mass or more, more preferably 80% by mass or more, further preferably 90% by mass or more, particularly preferably 95% by mass or more, and most preferably 98% by mass or more with respect to the amount of the thermoplastic resin composition. The thermoplastic resin composition forming the continuous filament may contain 100% by mass of the polybutylene adipate terephthalate resin.

The polybutylene adipate terephthalate resin is a biodegradable thermoplastic resin and is a copolymer of adipic acid, terephthalic acid, and butanediol. By having biodegradability, the polybutylene adipate terephthalate resin is expected to become one solution to problems arising from disposal of rubbish and problems regarding microplastics. The adipic acid, the terephthalic acid, and the butanediol do not need to be simultaneously copolymerized and may be copolymerized in multiple stages. In addition, the polybutylene adipate terephthalate resin is preferably a thermoplastic resin.

The polybutylene adipate terephthalate resin contains an adipic acid residue (adipic acid unit) and a terephthalic acid residue (terephthalic acid unit), and a molar ratio of the terephthalic acid residue to the adipic acid residue is preferably 1.0 or more and 3.0 or less. Regarding the lower limit of the molar ratio, the molar ratio is more preferably 1.1 or more and further preferably 1.2 or more. Meanwhile, regarding the upper limit of the molar ratio, the molar ratio is more preferably 2.5 or less and further preferably 2.0 or less. By the molar ratio being 1.0 or more, the repeated compression durability and the compression recoverability after heating compression at the usage environment temperature of the three-dimensional network structure are easily improved. Meanwhile, by the molar ratio being 3.0 or less, the flexibility is easily improved. Therefore, such a three-dimensional network structure is suitable as a cushioning material or the like.

The polybutylene adipate terephthalate resin has a melting point of preferably 125°C or more and 180°C or less. Regarding the lower limit of the melting point, the melting point is more preferably 130°C or more, further preferably 140°C or more, and even more preferably 145°C or more. Meanwhile, regarding the upper limit of the melting point, the melting point is more preferably 170°C or less and further preferably 160°C or less. By the melting point being 125°C or more, the repeated compression durability and the compression recoverability after heating compression at the usage environment temperature of the three-dimensional network structure are easily improved. Meanwhile, by the melting point being 180°C or less, the three-dimensional network structure easily exhibits an improved flexibility and is suitable as a cushioning material or the like.

The polybutylene adipate terephthalate resin has a melt flow rate (MFR) of preferably 3 g/10 min to 60 g/10 min. By the MFR being 3 g/10 min or more, the repeated compression durability and the compression recoverability after heating compression are easily improved. Regarding the lower limit of the MFR, the MFR is more preferably 4 g/10 min or more, further preferably 5 g/10 min or more, and even more preferably 6 g/10 min or more. Meanwhile, by the MFR being 60 g/10 min or less, the melt viscosity can be made high, and the fiber diameter of the continuous filament can be made large. Regarding the upper limit of the MFR, the MFR is more preferably 50 g/10 min or less, further preferably 40 g/10 min or less, and particularly preferably 30 g/10 min or less. The thermoplastic resin composition forming the continuous filament also preferably has an MFR within this range. The MFR of the resin can be measured through a method explained in EXAMPLES described later.

When using a commercially available resin as a polybutylene adipate terephthalate resin, in case where a resin has a low MFR, MFR of the resin can be increased by adding water to the resin to cause hydrolysis of the resin during melt extrusion. Meanwhile, in case where a resin has a high MFR, MFR of the resin can be reduced by drying the resin and then melt extruding.

The thermoplastic resin composition forming the continuous filament may include another biodegradable resin other than polybutylene adipate terephthalate resin. The biodegradable resin other than polybutylene adipate terephthalate resin preferably include polylactic acid, polylactic acid/polycaprolactone copolymer, polylactic acid/polyether copolymer, polyethylene terephthalate succinate, polybutylene succinate, polybutylene succinate adipate, polyglycolic acid, polycaprolactone, polyvinyl alcohol, cellulose acetate, and the like. These resins may be used alone or in combination. Details of the resins are shown in the positive list of green plastic (biodegradable plastic) with a classification number A-1 published by Japan BioPlastics Association. The thermoplastic resin composition forming the continuous filament may include a resin other than biodegradable resin. Examples of the resin include thermoplastic resins such as polyolefin, polyurethane, and polyester.

In addition, the thermoplastic resin composition forming the continuous filament may contain not only the polybutylene adipate terephthalate resin but also a resin having other copolymerization components other than adipic acid, terephthalic acid, and butanediol as units. Examples of the other copolymerization component include any dicarboxylic acid other than adipic acid and terephthalic acid, any diol other than butanediol, polyalkylene glycol, and a modifier for chain extension or end capping. These may be used alone or in combination.

Examples of the dicarboxylic acid other than adipic acid and terephthalic acid include oxalic acid, malonic acid, succinic acid, glutaric acid, pimelic acid, and suberic acid. These may be used alone or in combination.

Examples of the diol other than butanediol include methanediol, ethanediol, propanediol, pentanediol, and hexanediol. Example of the polyalkylene glycol include polymethylene glycol, polyethylene glycol, polypropylene glycol, and polybutylene glycol (polytetramethylene glycol). These may be used alone or in combination.

The modifier may be, for example, a polyisocyanate compound or a glycol compound. The polyisocyanate compound may be, for example, a diisocyanate compound.

Examples of the diisocyanate compound include hexamethylene diisocyanate, 4,4'-diphenylmethane diisocyanate, 2,4-tolylene diisocyanate, 2,6-tolylene diisocyanate, xylylene diisocyanate, 1,5-naphthylene diisocyanate, p-phenylene diisocyanate, isophorone diisocyanate, 4,4'-dicyclohexylmethane diisocyanate, tetra-methyl xylene diisocyanate, carbodiimide modified MDI, and polymethylene phenyl polyisocyanate. These compounds may be used alone or in combination.

As a monomer for synthesizing the thermoplastic resin composition forming the continuous filament, a petroleum-derived monomer may be used. However, biomass-derived monomers are preferable from the viewpoint of lowering environmental load. As to the biomass-derived monomers, for example, monomers shown in a positive list with a classification number A (biomass-derived plastic) published by Japan BioPlastics Association can be used.

The total amount of the adipic acid unit and the terephthalic acid unit contained per 100 mol% of the dicarbon units contained in the thermoplastic resin composition forming the continuous filament is preferably 70 mol% or more, more preferably 80 mol% or more, further preferably 90 mol% or more, even more preferably 95 mol% or more, and particularly preferably 99 mol% or more. The amount of the butanediol unit contained per 100 mol% of the diol units contained in the thermoplastic resin composition forming the continuous filament is preferably 70 mol% or more, more preferably 80 mol% or more, further preferably 90 mol% or more, even more preferably 95 mol% or more, and particularly preferably 99 mol% or more.

The thermoplastic resin composition forming the continuous filament may contain additives such as a deodorant agent, an antibacterial agent, an antifungal agent, an anti-mite agent, an anti-odor agent, an aromatic agent, a flame retardant, a moisture absorbing/releasing agent, an antioxidant, and a lubricant. These may be used alone or in combination. The total content of the various additives is preferably 5% by mass or less, more preferably 2% by mass or less, and further preferably 1% by mass or less with respect to 100% by mass of the thermoplastic resin composition.

### <Continuous Filament>

The three-dimensional network structure of the present invention has a three-dimensional random loop-bonded configuration and is made of a continuous filament made from the thermoplastic resin composition. The continuous filament is a linear filament having a continuous portion of at least 5 mm or more. Presence of a portion obtained by adhering intersections of such continuous filaments makes it easy to form a three-dimensional network structure. Therefore, the three-dimensional network structure preferably has an adhesion portion at which the intersections of the continuous filaments have been adhered to each other.

The continuous filament composing the three-dimensional network structure of the present invention may be a composite filament obtained by combination with another thermoplastic resin as long as the object of the present invention is achieved. Examples of the type of such a composite in the case of compositing the filament itself include composite filaments such as a sheath-core type, a side-by-side type, an eccentric sheath-core type, and the like.

One of the features of the three-dimensional network structure of the present invention is that an average fiber diameter of a surface layer portion is larger than an average fiber diameter of an inner layer portion in order to increase the surface stiffness of the three-dimensional network structure. Specifically, the average fiber diameter of the surface layer portion of the three-dimensional network structure of the present invention is not less than 1.05 times, preferably not less than 1.08 times, and more preferably not less than 1.10 times the average fiber diameter of the inner layer portion of the three-dimensional network structure. When the average fiber diameter of the surface layer portion is less than 1.05 times the average fiber diameter of the inner layer portion, a required surface stiffness and a required strength of contact points between the continuous filaments in the surface layer portion might not be able to be ensured, and a hardness retention rate necessary for cushion characteristics might not be able to be stably obtained. The upper limit of the ratio of the average fiber diameter of the surface layer portion to the average fiber diameter of the inner layer portion is not particularly limited, and the ratio is, for example, not more than 1.25 times. The average fiber diameter of the surface layer portion is 0.1 mm or more and 3.0 mm or less, preferably 0.2 mm or more and 2.5 mm or less, more preferably 0.3 mm or more and 2.0 mm or less, and further preferably 0.5 mm or more and 1.0 mm or less. The average fiber diameter of the inner layer portion is 0.1 mm or more and 3.0 mm or less, preferably 0.2 mm or more and 2.5 mm or less, more preferably 0.3 mm or more and 2.0 mm or less, and further preferably 0.5 mm or more and 1.0 mm or less. The average fiber diameter of the surface layer portion and the average fiber diameter of the inner layer portion can be measured through a method explained in EXAMPLES described later.

In the three-dimensional network structure of the present invention, the average fiber diameter differs between the surface layer portion and the inner layer portion, and thus it is difficult to exactly calculate an average fiber diameter of the entirety of the three-dimensional network structure (an average fiber diameter of the continuous filament forming the three-dimensional network structure). Thus, in the present specification, the average value of the two values, i.e., the average fiber diameter of the surface layer portion and the average fiber diameter of the inner layer portion, is defined as the average fiber diameter of the continuous filament forming the three-dimensional network structure. The average fiber diameter of the continuous filament forming the three-dimensional network structure of the present invention is 0.1 mm or more and 3.0 mm or less, preferably 0.2 mm or more and 2.5 mm or less, and more preferably 0.3 mm or more and 2.0 mm or less. When the average fiber diameter of the continuous filament is less than 0.1 mm, the continuous filament is excessively thin. Consequently, although favorable denseness and a favorably soft texture are obtained, it becomes difficult to ensure a hardness necessary for a three-dimensional network structure. Meanwhile, when the average fiber diameter of the continuous filament is more than 3.0 mm, although the hardness of the three-dimensional network structure can be sufficiently ensured, the network configuration might become rough, and other cushioning performances might become inferior. From such viewpoints, the average fiber diameter of the continuous filament needs to be set to fall within the appropriate range.

The continuous filament forming the three-dimensional network structure of the present invention preferably has an enthalpy of fusion of 16 J/g or more. By the enthalpy of fusion being 16 J/g or more, the compression recoverability after heating compression and the compression durabilities of the three-dimensional network structure can be improved. The enthalpy of fusion is more preferably 17 J/g or more, further preferably 18 J/g or more, even more preferably 19 J/g or more, still even more preferably 20 J/g or more, and particularly preferably 21 J/g or more. Meanwhile, the continuous filament forming the three-dimensional network structure of the present invention preferably has an enthalpy of fusion of 30 J/g or less. By the enthalpy of fusion being 30 J/g or less, the flexibility of the three-dimensional network structure can be improved, whereby noise that might be generated during compression and during recovery can be decreased. The enthalpy of fusion is more preferably 29 J/g or less, and further preferably 28 J/g or less.

An enthalpy (J/g) of an endothermic peak of the continuous filament forming the three-dimensional network structure of the present invention can be obtained from an integral value of an endothermic peak (melting peak) based on a DSC curve measured under a nitrogen atmosphere and at a heating rate of 20°C/min by using a differential scanning calorimeter, with a sample mass being set to 2.0 mg±0.1 mg. The integral value can be obtained as follows. That is, a point at which the curve related to the aforementioned endothermic peak (melting peak) starts to be away from a baseline on the low-temperature side is defined as a start point, a point at which the curve starts to be in contact with a baseline on the high-temperature side is defined as an end point, a straight line connecting the start point and the end point is drawn, and integration is performed on the portion enclosed by the straight line and the curve. An example of the DSC curve is shown in FIG. 1. A broken line in FIG. 1 is the straight line connecting the above start point and the above end point of the endothermic peak (melting peak), and the portion enclosed by the broken line and the curve is an integration region on which integration is performed.

The enthalpy of the endothermic peak, in which the DSC curve regarding the continuous filament composing the three-dimensional network structure measured by using a differential scanning calorimeter has a minimum value in a range from 30°C to 70°C, is 2.5 J/g or less. The "enthalpy of the endothermic peak in which the DSC curve has a minimum value in the range from 30°C to 70°C" is sometimes expressed as a low-temperature phase enthalpy in the present invention. By the low-temperature phase enthalpy being 2.5 J/g or less, the 40°C-compression residual strain is decreased. As a result, feeling of irrecoverable deformation when the three-dimensional network structure is used as a cushioning material can be decreased. Considering this advantage, the low-temperature phase enthalpy is preferably 1.5 J/g or less, and more preferably 1.0 J/g or less. The lower limit of the low-temperature phase enthalpy is not particularly limited, but the low-temperature phase enthalpy is, for example, 0.2 J/g or more in consideration of technical difficulties.

### <Three-Dimensional Network Structure>

The three-dimensional network structure of the present invention favorably has a single-layer configuration but may have a multi-layer configuration as long as the object of the present invention is achieved. Examples of the method for obtaining such a multi-layer configuration include: a method in which such three-dimensional network structures are stacked on each other and fixed using a fabric or the like; a method in which such three-dimensional network structures are melted and fastened through heating; a method in which such three-dimensional network structures are adhered using an adhesive; a method in which such three-dimensional network structures are restrained through sewing or using a band or the like; and the like.

The cross-sectional shape of the continuous filament forming the three-dimensional network structure of the present invention is not particularly limited, but setting the continuous filament to have a hollow cross section or an atypical cross section makes it possible to impart preferable resistance to compression and texture.

The shape of the three-dimensional network structure of the present invention is not particularly limited. Examples of the shape of the three-dimensional network structure include a plate, triangular, quadrangular such as polygonal, cylindrical, spherical shape, or combinations thereof. The three-dimensional network structure may be obtained by molding with baffles when resin is melt extruded, or may be molded by a method such as cutting or hot pressing.

The three-dimensional network structure of the present invention has an apparent density of preferably 0.01 g/cm³ to 0.20 g/cm³. By the apparent density being 0.01 g/cm³ or more, the hardness of the three-dimensional network structure is improved. As a result, bottoming-out feeling perceived when the three-dimensional network structure is used as a cushion or the like can be decreased. Thus, regarding the lower limit of the apparent density, the apparent density is more preferably 0.02 g/cm³ or more, further preferably 0.025 g/cm³ or more, and particularly preferably 0.03 g/cm³ or more.

Meanwhile, when the apparent density is 0.20 g/cm³ or less, the three-dimensional network structure exhibits an improved flexibility and can be suitably used as a cushioning material or the like. Thus, regarding the upper limit of the apparent density, the apparent density is more preferably 0.15 g/cm³ or less and further preferably 0.10 g/cm³ or less. The apparent density of the three-dimensional network structure can be measured through a method explained in EXAMPLES described later.

The three-dimensional network structure of the present invention has a thickness of preferably 10 mm to 300 mm. By the thickness being 10 mm or more, the three-dimensional network structure is easily used as a cushioning material or the like. Considering this, regarding the lower limit of this thickness, the thickness is more preferably 15 mm or more, further preferably 20 mm or more, and particularly preferably 25 mm or more. Meanwhile, regarding the upper limit of this thickness, the thickness is more preferably 200 mm or less, further preferably 150 mm or less, and particularly preferably 100 mm or less in consideration of the size of a manufacturing apparatus. The thickness of the three-dimensional network structure can be measured through a method explained in EXAMPLES described later.

The three-dimensional network structure of the present invention has a 40°C-compression residual strain of preferably 25% or less. Consequently, the compression recoverability after heating compression can be improved. Regarding the upper limit of the 40°C-compression residual strain, the 40°C-compression residual strain is more preferably 20% or less and further preferably 15% or less. The 40°C-compression residual strain is not particularly limited and may be, for example, 1% or more and 5% or more. The 40°C-compression residual strain can be measured through a method explained in EXAMPLES described later.

The three-dimensional network structure of the present invention has a 25%-compression hardness of preferably 10 N/φ200 to 600 N/φ200, more preferably 30 N/φ200 to 400 N/φ200, and further preferably 50 N/φ200 to 200 N/φ200. When the 25%-compression hardness is less than 10 N/φ200, bottoming-out feeling might be perceived. Meanwhile, when the 25%-compression hardness is more than 600 N/φ200, the three-dimensional network structure might become excessively hard, and the cushioning properties thereof might be impaired.

The three-dimensional network structure of the present invention has a 40%-compression hardness of preferably 40 N/φ200 to 1000 N/φ200, more preferably 60 N/φ200 to 700 N/φ200, and further preferably 80 N/φ200 to 400 N/φ200. When the 40%-compression hardness is less than 40 N/φ200, bottoming-out feeling might be perceived. Meanwhile, when the 40%-compression hardness is more than 1000 N/φ200, the three-dimensional network structure might become excessively hard, and the cushioning properties thereof might be impaired.

The three-dimensional network structure of the present invention has a 65%-compression hardness of preferably 80 N/φ200 to 2000 N/φ200, more preferably 100 N/φ200 to 1000 N/φ200, and further preferably 150 N/φ200 to 600 N/φ200. When the 65%-compression hardness is less than 80 N/φ200, bottoming-out feeling might be perceived. Meanwhile, when the 65%-compression hardness is more than 2000 N/φ200, the three-dimensional network structure might become excessively hard, and the cushioning properties thereof might be impaired.

The three-dimensional network structure of the present invention has a residual strain after 750-N constant load repeated compression of 15% or less and preferably 10% or less. When the residual strain after 750-N constant load repeated compression is more than 15%, use for a long period leads to decrease in the thickness of the three-dimensional network structure, and such a three-dimensional network structure is not preferable as a cushioning material. In the present specification, the "750-N constant load repeated compression" means repeatedly compressing the three-dimensional network structure at a constant load of 750 N, and the "residual strain after 750-N constant load repeated compression" means a thickness, of the three-dimensional network structure, decreased by performing the above repeated compression. The lower limit value of the residual strain after 750-N constant load repeated compression is not particularly limited, but, in the case of the three-dimensional network structure obtained in the present invention, this residual strain is 0.1% or more.

The three-dimensional network structure of the present invention has a 40%-compression hardness retention rate after 750-N constant load repeated compression of 45% or more, preferably 48% or more, and more preferably 50% or more. When the 40%-compression hardness retention rate after 750-N constant load repeated compression is less than 45%, use for a long period leads to decrease in the firmness of the cushioning material, whereby significant change in the firmness might be perceived. The upper limit value of the 40%-compression hardness retention rate after 750-N constant load repeated compression is not particularly limited, but, in the case of the three-dimensional network structure obtained in the present invention, this hardness retention rate is 95% or less.

The three-dimensional network structure of the present invention has a 65%-compression hardness retention rate after 750-N constant load repeated compression of 60% or more, preferably 63% or more, and more preferably 65% or more. When the 65% hardness retention rate after 750-N constant load repeated compression is less than 60%, use for a long period leads to decrease in the firmness of the cushioning material, whereby bottoming-out feeling might be perceived. The upper limit value of the 65%-compression hardness retention rate after 750-N constant load repeated compression is not particularly limited, but, in the case of the three-dimensional network structure obtained in the present invention, this hardness retention rate is 99% or less.

The three-dimensional network structure of the present invention is preferably characterized by having a 40%-compression hardness retention rate after 750-N constant load repeated compression of 45% or more and a 65%-compression hardness retention rate after 750-N constant load repeated compression of 60% or more. Setting the hardness retention rates to fall within the above ranges is essential for obtaining a three-dimensional network structure that sustains, after being used for a long period, little change in the hardness of the three-dimensional network structure and little change in comfort in sitting and comfort in sleeping and that can be comfortably used for a long period. A durability test involving the 750-N constant load repeated compression is a test for evaluating a durability even higher than in a 50%-constant displacement repeated compression test having attracted attention in prior art documents and the like to date. The reason is as follows. In the 50%-constant displacement repeated compression test, the compression amount is fixed at 50% of a thickness from start of processing to end of the processing. Meanwhile, in the case of the durability test involving 750-N constant load repeated compression, for example, even when the load of 750 N corresponds to a displacement of 50% of the thickness upon start of repeated compression processing, the hardness gradually decreases during the processing, and thus the compression amount exceeds 50% of the thickness at the end of the processing, whereby the amount of deformation sustained by the sample during the test becomes larger than in the 50%-constant displacement repeated compression test.

The three-dimensional network structure of the present invention has a compressive deflection coefficient of preferably 2.5 or more, more preferably 2.8 or more, and further preferably 3.0 or more. When the compressive deflection coefficient is less than 2.5, comfort in sitting or comfort in sleeping on the cushioning material might be impaired. By setting the compressive deflection coefficient to fall within the above range, a three-dimensional network structure on which comfort in sitting and comfort in sleeping are satisfactory is obtained. In particular, it is found that, when the hardnesses become comparatively high, setting the compressive deflection coefficient to fall within the above range leads to satisfactory comfort in sitting and comfort in sleeping. The compressive deflection coefficient is a value resulting from dividing the 65%-compression hardness by the 25%-compression hardness, and the compressive deflection coefficient can be made large by either decreasing the 25%-compression hardness or increasing the 65%-compression hardness. The mechanism in which the compressive deflection coefficient is enhanced in the present invention has not been sufficiently clarified, but the enhancement is inferred to be probably because: the surface layer portion of the three-dimensional network structure of the present invention has a large fiber diameter, and this three-dimensional network structure has a high surface stiffness and a high 65%-compression hardness. This advantageous effect is inferred to enable stable increase in the compressive deflection coefficient. The upper limit value of the compressive deflection coefficient is not particularly limited, but, in the case of the three-dimensional network structure obtained in the present invention, this compressive deflection coefficient is 8.0 or less.

The present inventors have found that, in order to obtain a three-dimensional network structure that retains the hardnesses in the durability test involving 750-N constant load repeated compression, it is necessary to achieve: a feature of receiving an externally applied load (750 N) at the surface layer portion of the three-dimensional network structure and dispersing the load through the surface layer as a surface to mitigate burden on the inner layer; and a feature of keeping the load-dispersing effect of the surface layer as a surface also during the test involving constant load repeated compression. Causing the surface layer portion and the inner layer portion to have different configurations is essential for achieving the former feature, and strengthening the strength of the contact points between the continuous filaments present in the surface layer portion is essential for achieving the latter feature. That is, the differences between a conventionally known three-dimensional network structure having a low 50%-constant displacement repeated compression strain and the three-dimensional network structure of the present invention are as follows. In the three-dimensional network structure of the present invention, fusion between the continuous filaments forming the three-dimensional network structure is made firmer to strengthen the strength of the contact points between the continuous filaments. Along with this, the average fiber diameter of the surface layer portion of the three-dimensional network structure is made larger than the average fiber diameter of the inner layer portion of the three-dimensional network structure, the surface layer portion and the inner layer portion are caused to have different configurations, and the area of the contact points between the continuous filaments is made large to cause the strength of the contact points to become higher in the surface layer portion of the three-dimensional network structure than in the inner layer portion of the three-dimensional network structure. Consequently, fracture of the contact points that occurs during repeated compression processing is further suppressed, whereby the effect of surface dispersion, through the surface layer portion, of the load (750 N) received during the repeated compression is kept being exhibited. Since it is difficult to achieve the feature of setting the 40% hardness retention rate after 750-N constant load repeated compression to be stably 45% or more just by strengthening the strength of the contact points between the continuous filaments forming the three-dimensional network structure, the fibers of the surface layer are selectively thickened to increase the surface stiffness, the strength of the contact points between the filaments in the surface layer is designed to be high, and the inner layer and the surface layer are caused to have different configurations, thereby being able to stably achieve this feature.

The feature of causing the surface layer portion and the inner layer portion to have different configurations and the feature of strengthening the strength of the contact points between the continuous filaments in the surface layer portion are necessary for obtaining the three-dimensional network structure of the present invention as described above and are achieved by setting the average fiber diameter of the surface layer portion to be not less than 1.05 times the average fiber diameter of the inner layer portion. In a case where the average fiber diameter of the surface layer portion is less than 1.05 times the average fiber diameter of the inner layer portion, the difference in configuration between the surface layer portion and the inner layer portion is small, and a required surface stiffness is not obtained. Therefore, the effect of surface dispersion, through the surface layer portion, of the load received during repeated compression decreases, and sufficient hardness retention rates cannot be obtained. A prior art document describing a network structure in which a soft layer having a small fiber diameter and a durable inner layer having a large fiber diameter are respectively provided as a surface and a base layer to enhance cushioning properties and durability has been known. Meanwhile, in the present invention, the fiber diameter of the surface layer is made large to increase the surface stiffness and improve the hardness retention rates. Thus, the present invention is based on a design concept fundamentally different from that of the prior art document. With the aforementioned manufacturing method, the conventional 50%-constant displacement repeated compressibility is excellent, but the durability after harsher 750-N constant load repeated compression on which the present invention focuses is not necessarily excellent, and thus it has been difficult to achieve the repeated compression characteristics required in the present invention.

The three-dimensional network structure is preferably free from a bonding promoter. The absence of a bonding promoter prevents excessive hardening generated by excessive bonding due to bonding promoter in the three-dimensional network structure. In addition, a decrease in fineness of the three-dimensional network structure caused by excessively increased bonding area per one contact point may be prevented. Examples of the bonding promoter include polycaprolactone, polybutylene succinate, polybutylene sebacate terephthalate, and polybutylene azelate terephthalate.

The three-dimensional network structure may be colored. A color agent such as a pigment or a dye can be used. The color agent may be contained in the resin before melt spinning, or the continuous filaments may be coated with a color agent by immersion or application after the formation of the three-dimensional network structure.

The three-dimensional network structure of the present invention is preferably applied to a cushion. The cushion may be resilient enough to support objects or may be able to reduce impact. Examples of the cushion include cushions for office chairs, furniture, sofas, bedding such as beds, cushions for seats of vehicles such as trains, automobiles, two-wheeled vehicles, child safety seats, and baby buggies, shock-absorbing mats such as floor mats and members for preventing collision and nipping.

### <Manufacturing Method for Three-dimensional Network Structure>

A manufacturing method for the three-dimensional network structure of the present invention preferably includes: an extrusion step of extruding, from a nozzle, the thermoplastic resin composition melted; a molding step of molding the continuous filament made from the thermoplastic resin composition extruded from the nozzle, into a three-dimensional network configuration so as to obtain a molded body; and a heat treatment step of heat treating the molded body. A three-dimensional network structure for which the heat treatment step has not been finished is referred to as a molded body in order to avoid confusion with a three-dimensional network structure as a finished product (a three-dimensional network structure for which the heat treatment step has been finished). An example of the extrusion step and the molding step is described below, but the method is not limited thereto.

First, the thermoplastic resin composition including polybutylene adipate terephthalate resin with a melting point of Tm (°C) is distributed from a multi-row nozzle having a plurality of orifices having a plurality of different orifice hole diameters (to be described later), and then discharged downward from the nozzle at a spinning temperature of Tm + 20°C or higher and lower than Tm + 180°C (preferably Tm + 75°C or higher and lower than Tm + 120°C). Next, a three-dimensional network structure is formed by bringing continuous filaments into contact with each other in a melt state and fusing contact portions thereof, then the structure is sandwiched with take-up conveyors and cooled with cooling water in a water tank. After cooling, the solidified molded body is drawn, then drained or dried, and the molded body having two or one smoothed side can be obtained. With regard to the spinning process and the cooling process, for example, descriptions in Japanese Laid-Open Patent Publication No. H7-68061 can be referenced. In case where only one surface needs to be smoothed, continuous filaments are discharged on an inclined take-up net, and the continuous filaments are contacted with each other and fused at contact portions thereof in a melt state. While the three-dimensional network structure is being formed, the shape only on the take-up net touching side of the structure may be loosened and the structure may be cooled. The obtained molded body may be subjected to a heat treatment. The drying treatment of the molded body may be the heat treatment.

Water may be added to the thermoplastic resin composition before the resin is discharged from a nozzle. Adding water to the thermoplastic resin composition allows promoted degradation of the thermoplastic resin composition in the production process of the three-dimensional network structure or improvement in flexibility of the resin and can reduce the difference in compression durability regardless of which surface is pressurized. In addition, water is added preferably at 2.0% by mass or less with respect to the thermoplastic resin composition, thereby enabling prevention of excessive degradation of the thermoplastic resin composition in the production process of the three-dimensional network structure and thus facilitating improvement in compression recovery after heating compression and compression durability from both sides. Water may be added to the thermoplastic resin composition in any manner. For example, the thermoplastic resin composition may be absolutely dried in vacuum at 100°C for 12 hours or more before discharged from a nozzle, and a predetermined amount of water may be added with respect to 100% by mass of absolutely dried thermoplastic resin composition.

The melt flow rate (MFR) of the polybutylene adipate terephthalate resin is preferably lower than a desired MFR of the continuous filament forming the three-dimensional network structure by 0.5 g/10 min or more and less than 20.0 g/10 min before melt-extrusion. Thermal degradation or shear degradation of the resin is induced during melt-extrusion, and thus the MFR before melt-extrusion is controlled to be as described above. By doing so, a continuous filament having the desired MFR is easily obtained.

In order to obtain the three-dimensional network structure of the present invention, fusion between the continuous filaments of the three-dimensional network structure to be obtained needs to be made firm to strengthen the strength of the contact points between the continuous filaments. As a result of strengthening the strength of the contact points between the continuous filaments forming the three-dimensional network structure, the repeated compression durability of the three-dimensional network structure can be improved.

One means for obtaining a three-dimensional network structure having a strengthened strength of contact points is, for example, preferably increasing the spinning temperature of the thermoplastic resin. The spinning temperature differs depending on the characteristics of the resin but is preferably Tm+30°C or higher and Tm+150°C or lower, more preferably Tm+40°C or higher and Tm+140°C or lower, further preferably Tm+50°C or higher and Tm+130°C or lower, and particularly preferably Tm+75°C or higher and lower than Tm+120°C.

One of suitable methods for causing the surface layer portion and the inner layer portion to have different fiber diameters in the three-dimensional network structure of the present invention is a method in which only fibers near the surface of the three-dimensional network structure are cooled early to increase the fiber diameter of the surface layer portion alone.
There is a method for obtaining different fiber diameters by a nozzle configuration in which the hole diameters of the nozzle are changed between a surface layer portion and an inner layer portion to increase the fiber diameter of the surface layer portion alone as is known in a prior art document. Such a method has the following disadvantages. A strain of the loop shape of the surface layer portion or a difference in density between the surface layer portion and the inner layer portion becomes obvious, i.e., a problem arises in terms of appearance quality. In addition, it is easy for the surface layer portion and the inner layer portion to be extruded in an unbalanced manner, or stability in manufacturing and manufacturing of uniform products become difficult to achieve, i.e., a problem arises in terms of manufacturing. In addition, it is difficult to obtain a three-dimensional network structure having excellent durability after 750-N constant load repeated compression, which is expected to be attained in the present invention.

As the method in which only the fibers near the surface of the three-dimensional network structure are cooled, there are a method in which the ambient temperature is set to be low and a method in which cooling air is selectively applied to the surface. In the present specification, the "ambient temperature" refers to a temperature measured by a thermometer that is present in the same space as that of a spinning machine, is located at a distance of 1 m or more and less than 1.5 m from the spinning machine, and is located at a height from an extrusion surface to a water surface. In the case of cooling the fibers of the surface layer at the ambient temperature, the ambient temperature is preferably 50°C or lower, more preferably 40°C or lower, and further preferably 35°C or lower. The ambient temperature is preferably -10°C or higher from the viewpoint of preventing significant decrease in the strength of the contact points. In the case of selectively applying cooling air to the surface, the temperature of the cooling air is preferably not more than the melting point of the resin and preferably not less than the ambient temperature. Also, designing is preferably performed such that: cooling air is caused to flow downward by an entrained flow on the surface; or, even when cooling air penetrates to the inner layer, the penetrating air has an increased temperature as a result of undergoing heat exchange with the surface fibers so as not to decrease the strength of contact points of the inner layer. From such viewpoints, the cooling in the fiber direction is preferably performed moderately. The air speed of the cooling air is preferably 0.3 m/second or less or more preferably 0.2 m/second or less. By employing one of the above methods or combining two or more of the above methods, the fiber diameter of the surface layer portion can be made larger than the fiber diameter of the inner layer portion.

A device for applying cooling air preferably has a configuration in which cooling air is applied in the thickness direction of the three-dimensional network structure from one surface or both surfaces thereof so as to cover the entirety thereof in the width direction. The device for applying cooling air can be selected as appropriate according to the three-dimensional network structure to be obtained. The installation location in the height direction of the device for applying cooling air may be any location and the height of the device may be changed as necessary, as long as the installation location is between the nozzle surface and the cooling water. The height does not have to be entirely even in the width direction and may be changed depending on a portion. It is also allowable to apply cooling air only to a portion at which the surface is to be more firmly formed. Also, it is also allowable to, according to use, apply cooling air only to one surface or apply cooling air from all the surfaces in the thickness direction of the three-dimensional network structure. At least one flow-regulating portion such as a wire net is preferably provided in order to cause the air speed of the cooling air to become as even as possible. In the case of increasing the temperature of the cooling air, a hot air generation device is preferably used, and waste heat near the nozzle may be used.

The three-dimensional network structure of the present invention is preferably obtained by means of optimizing a nozzle shape, a dimension, and the arrangement of nozzle holes. Regarding the nozzle shape, the diameters of orifices for forming thin fibers are preferably 1.5 mm or less, and the diameters of orifices for forming thick fibers are preferably 2 mm or more. Also, the nozzle orifices for forming thick fibers preferably have hollow-forming shapes, and examples of the nozzle with such a shape include C-type nozzles, nozzles having triple-bridge shapes, and the like. Among these nozzles, nozzles having triple-bridge shapes are preferable from the viewpoint of resistance to pressure. An inter-hole pitch of the orifices for forming thin fibers and an inter-hole pitch of the orifices for forming thick fibers are each preferably 4 mm or more and 12 mm or less and more preferably 5 mm or more and 11 mm or less. Examples of the arrangement of nozzle holes include lattice arrangement, circumferential arrangement, staggered arrangement, and the like, and lattice arrangement or staggered arrangement is preferable from the viewpoint of the appearance quality of the three-dimensional network structure. Here, each of the inter-hole pitches is the distance between the centers of nozzle holes.

After melt-molding, the polybutylene adipate terephthalate resin is cooled preferably with cooling water. The polybutylene adipate terephthalate resin may shrink in molding by the time the resin is solidified by cooling. Because of the molding shrinkage phenomenon, the three-dimensional network structure should preferably be formed to have a width and a thickness in consideration of molding shrinkage. For example, by lowering the solidification temperature of melting resin, the shrinkage in molding can be reduced. Therefore, the temperature of the cooling water in the water tank is preferably 20°C or lower, more preferably 15°C or lower, and particularly preferably 10°C or lower. The resin is preferably cooled with cooling water with the cooling time of preferably 30 seconds or more. The resin is preferably solidified by cooling in a water tank.

The heat treatment may be conducted in a commercially available hot-air drying oven or may be in a warm water bath. The heat treatment temperature is preferably 50°C or higher. The heat treatment under such conditions can increase an enthalpy of fusion. The heat treatment temperature is more preferably 60°C or higher, and further preferably 70°C or higher. The heat treatment may be performed multiple times at different temperatures.

The heat treatment time in the heat treatment step is preferably 1 minute or more. This can increase an enthalpy of fusion. The heat treatment time is more preferably 5 minutes or more, further preferably 10 minutes or more, and particularly preferably 15 minutes or more. Meanwhile, the upper limit of the heat treatment time in each heat treatment step is preferably 60 minutes or less, and more preferably 50 minutes or less.
This can reduce yellowing, odor, and molecular weight loss of polybutylene adipate terephthalate resin due to polymer decomposition and degradation in the heat treatment step. Further, productivity can be also improved. If heat treatment is performed multiple times, it is preferable that total heat treatment time fall within the above range.

The molded body solidified by cooling in the water tank may be kept under given temperature in the range of 20°C to 50°C for 1 minute or more before heat treatment. In heat treatment, the thickness of the molded body may change in some cases due to its own weight, however, the change in thickness of the molded body can be reduced by keeping the molded body in the range of 20°C to 50°C after solidification by cooling. For example, after solidification by cooling in a water tank, the molded body may be dried with a continuous dryer which has a first area of a hot air oven to keep the molded body at relative low temperature and a subsequent area of the hot air oven to heat treatment the molded body at relative high temperature.

Additives that can impart functions such as a deodorant and antibacterial property, an antifungal property, an anti-mite property, an anti-odor property, an aromatic property, a flame-retardant property, and a moisture absorbing/releasing property may be added to the thermoplastic resin in any step from the production step of the thermoplastic resin used as a raw material for three-dimensional network structure to the molding step of the three-dimensional network structure. In manufacturing the three-dimensional network structure, functional additives such as an antioxidant and a lubricant may be added to the polybutylene adipate terephthalate resin as a raw material. The functional additives may be used alone or in combination. Depending on the color tone and quality of the resin after being melted, it is preferable to mix various functional additives into a resin during melt extrusion to adjust the content of the functional additives.

Examples of the antioxidant include known phenol-based antioxidant, phosphite-based antioxidant, thioether-based antioxidant, benzotriazole-based UV absorber, triazine-based UV absorber, benzophenone-based UV absorber, N-H type hindered amine-based light stabilizer, and N-CH₃ type hindered amine-based light stabilizer.

Examples of the phenol-based antioxidant include 1,3,5-tris[[3,5-bis(1,1-dimethylethyl)-4-hydroxyphenyl]methyl]-1,3,5-triazine-2,4,6(1H,3H,5H)-trione, 1,1,3-tris(2-methyl-4-hydroxy-5-tert-butylphenyl)butane, 4,4'-butylidenebis(6-tert-butyl-m-cresol), 3-(3,5-di-tert-butyl-4-hydroxyphenyl)propionic acid stearyl, pentaerythritol tetrakis[3-(3,5-di-tert-butyl-4-hydroxyphenyl)propionate], Sumilizer AG 80, and 2,4,6-tris(3',5'-di-tert-butyl-4'-hydroxybenzyl)mesitylene.

Examples of the phosphite-based antioxidant include 3,9-bis(octadecyloxy)-2,4,8,10-tetraoxa-3,9-diphosphaspiro[5,5]undecane, 3,9-bis(2,6-di-tert-butyl-4-methylphenoxy)-2,4,8,10-tetraoxa-3,9-diphosphaspiro[5,5]undecane, 2,4,8,10-tetrakis(1,1-dimethylethyl)-6-[(2-ethylhexyl)oxy]-12H-dibenzo[d,g][1,3,2]dioxaphosphocin, tris(2,4-di-tert-butylphenyl)phosphite, tris(4-nonylphenyl)phosphite, 4,4'-isopropylidenediphenol C12-15 alcohol phosphite, diphenyl(2-ethylhexyl)phosphite, diphenyl isodecyl phosphite, triisodecyl phosphite, and triphenyl phosphite.

Examples of the thioether-based antioxidant include bis[3-(dodecylthio)propionate]2,2-bis[[3-(dodecylthio)-1-oxopropyloxy]methyl]-1,3-propanediyl and 3,3'-ditridecyl thiobispropionate.

In order to prevent thermal degradation of the thermoplastic resin, a mixture of phenol-based antioxidant and a phosphite-based antioxidant may be used. When these two types of antioxidants are used, the total content of these two types of antioxidants is preferably 0.05% by mass or more and 1.0% by mass or less with respect to 100% by mass of the thermoplastic resin composition.

Examples of the lubricant include hydrocarbon-based waxes, higher alcohol-based waxes, amide-based waxes, ester-based waxes, and metal soap. The lubricant is added, if needed, at 0.5% by mass or less with respect to 100% by mass of the thermoplastic resin composition on a mass basis.

The present application claims benefit of priority to Japanese Patent Application No. 2023-165925 filed on September 27, 2023. The entire contents of the specification of Japanese Patent Application No. 2023-165925 filed on September 27, 2023 are incorporated herein by reference.

### EXAMPLES

Hereinafter, the present invention will be specifically described with Examples. However, the scope of the present invention is not limited by the following Examples. The present invention can be carried out with modifications within a range conforming to the gist described above and/or below, and all of which are included in the technical scope of the present invention.

The characteristic values of the three-dimensional network structure in Examples 1 to 5 and Comparative Examples 1 to 2 were measured by the following methods. The sample size described below was the standard size for the measurement, however, a sample in available size was alternatively used in case of insufficiency in sample size.

### (1) Average Fiber Diameter

A sample was cut into a size of 10 cm×10 cm, and filaments (fibers) having a length of about 5 mm were collected from 10 locations in each of the surface layer portion and the inner layer portion of the three-dimensional network structure. The fibers of the surface layer portion were collected from the outermost layer in the thickness direction of the three-dimensional network structure, i.e., a fiber portion outside of which no fibers were present. The fibers of the inner layer portion were collected from within a range occupying 30% of the thickness of the three-dimensional network structure with the center of the range being the center in the thickness direction of the three-dimensional network structure (within a range from a point corresponding to 35% in the thickness direction from one surface to a point corresponding to 65% in the thickness direction from the one surface). The fiber diameters of the filaments collected from 10 locations in each of the surface layer portion and the inner layer portion were measured with the focus of an optical microscope being placed on a fiber diameter measurement portion at an appropriate magnification. The average value of the fiber diameters obtained from the fibers of the surface layer portion was regarded as an average fiber diameter of the surface layer portion, and the average value of the fiber diameters obtained from the fibers of the inner layer portion was regarded as an average fiber diameter of the inner layer portion. Then, the average value of the two values, i.e., the average fiber diameter of the surface layer portion and the average fiber diameter of the inner layer portion, was regarded as an average fiber diameter of the entirety of the sample.

### (2) Thickness and Apparent Density

Each of the three-dimensional network structures was cut into a size of 10 cm×10 cm in the longitudinal and lateral directions, and the obtained sample was left at rest for 24 hours under no load. Thereafter, a test piece thickness meter (model "FD-80N" manufactured by KOBUNSHI KEIKI CO., LTD.) was used to measure the height at one location which was the center of the sample, and this height of the sample was regarded as a thickness of the three-dimensional network structure. Furthermore, the sample was placed on an electronic balance, and the weight of the sample was measured. The height of the sample was multiplied by the area (100 cm²) defined by the longitudinal and lateral sides of the sample to obtain a volume of the sample, and the weight of the sample was divided by the volume to obtain an apparent density. The aforementioned operation was performed three times, and average values (n=3) of the thicknesses and the apparent densities of the three-dimensional network structure were obtained.

### (3) Molar Ratio of Terephthalic Acid Residue to Adipic Acid Residue of Polybutylene Adipate Terephthalate Resin

The molar ratio of the terephthalic acid residue to the adipic acid residue of each of polybutylene adipate terephthalate resins was measured through ¹H-NMR at a resonance frequency of 600 MHz. The NMR device AVANCE-NEO 600 manufactured by Bruker Corporation was used as a measurement device, and measurement was performed as follows.
10 to 15 mg of a sample was dissolved in a solvent in which the volume ratio of deuterated chloroform to trifluoroacetic acid was 85/15. Then, an NMR tube was filled with the resultant solution, and measurement was performed. Deuterated chloroform was used as a lock solvent, the standby time was set to 1 second, the data acquisition time was set to 4 seconds, and the number of times of integration was set to 64 times.

When the peak of chloroform is set to 7.28 ppm, the peak of adipic acid is detected at 2.45 ppm, and the peak of terephthalic acid is detected at 8.15 ppm.

When the peak integral value of adipic acid is represented by a and the peak integral value of terephthalic acid is represented by b, the molar ratio of the terephthalic acid residue to the adipic acid residue of the polybutylene adipate terephthalate resin can be expressed by the following formula. $Molar ratio = \left(\left(b/4\right)/\left(a/4\right)\right)$

### (4) Melting Point (Tm)

Resin pellets were collected as a sample and weighed out such that the mass of the sample was 2.0 mg ± 0.1 mg. Then, measurement was performed by using a differential scanning calorimeter (Discovery DSC25 manufactured by TA Instruments Corporation) under a condition of a nitrogen atmosphere at a temperature increase rate of 20°C/min, to obtain a DSC curve. From the DSC curve, a temperature in an endothermic peak (melting peak) was obtained. The above operation was performed 3 times, and the average value of the melting points was obtained (n=3).

### (5) Enthalpy of fusion

A sample was collected from each of the three-dimensional network structures and weighed out such that the mass of the sample was 2.0 mg ± 0.1 mg. Then, measurement was performed by using the differential scanning calorimeter (Discovery DSC25 manufactured by TA Instruments Corporation) under a condition of a nitrogen atmosphere at a temperature increase rate of 20°C/min, to obtain a DSC curve. From the DSC curve, an integral value of an endothermic peak (melting peak) was obtained, thereby evaluating an enthalpy of fusion (J/g).

The integral value of the endothermic peak (melting peak) was obtained as follows. That is, a point at which a curve related to the endothermic peak (melting peak) started to be away from the low-temperature side of a baseline was defined as a start point, a point at which the curve started to be in contact with the high-temperature side of the baseline was defined as an end point, a straight line connecting the start point and the end point was drawn, and a region enclosed by the straight line and the curve was integrated to obtain the enthalpy of fusion. The above operation was performed 3 times, and the average value of the melting enthalpies was obtained (n=3). The above start point was regarded as a melting-start onset temperature (°C).

### (6) Low-temperature Phase Enthalpy

In the DSC curve in the above item (5), an enthalpy of an endothermic peak in which the DSC curve had a minimum value in the range from 30°C to 70°C was obtained, and this enthalpy was defined as a low-temperature phase enthalpy. An integral value of the endothermic peak in the low-temperature phase region was obtained as follows. That is, a point at which a curve related to the endothermic peak started to be away from the low-temperature side of a baseline was defined as a start point, a point at which the curve started to be in contact with the high-temperature side of the baseline was defined as an end point, a straight line connecting the start point and the end point was drawn, and a region enclosed by the straight line and the curve in the range from 30°C to 70°C was integrated to obtain the low-temperature phase enthalpy. The above point (start point) where the curve started to be away from the low-temperature side of a baseline was regarded as a low-temperature phase onset temperature (°C). The above operation was performed 3 times, and the average value of the low-temperature phase enthalpies was obtained (n=3). An example of the experiment data is shown in FIG. 1.

### (7) Melt Flow Rate (MFR)

The polybutylene adipate terephthalate resin was dried in a vacuum at 80°C for 2 hours or more. Then, a melt flow rate (MFR) was quickly measured such that absorption of water in air was prevented as much as possible. The melt flow measurement was performed according to ISO 1133 by using the Melt Indexer F-F01 manufactured by Toyo Seiki Seisaku-sho, Ltd. The measurement temperature was set to 190°C, and the load was set to 2.16 kg. The above operation was performed 3 times, and the average value of the melt flow rates was obtained (n=3).

### (8) 40°C-Compression Residual Strain

Each of the three-dimensional network structures was cut into a size of 10 cm×10 cm. Then, a pre-processing thickness (c) of the obtained sample was measured through the method described in the above (2). The sample, the thickness of which was measured, was sandwiched between jigs capable of holding the sample in a 50%-compressed state, was put into a dryer controlled to be at 40°C, and was left at rest for 22 hours. Thereafter, the sample was taken out, was cooled to eliminate compressive strain, and was left at rest for 30 minutes.

Then, a thickness (d) of the sample was measured. These thicknesses were inputted to the following formula to obtain a 40°C-compression residual strain. The aforementioned operation was performed three times, and an average value (n=3) of the 40°C-compression residual strains was obtained. $40 ° C - compression residual strain \left(%\right) = \left\{\left(c\right)-\left(d\right)/c\right\} \times 100$

### (9) 25%, 40%, and 65%-Compression Hardnesses and Compressive Deflection Coefficient

Each of the three-dimensional network structures was cut into a size of 40 cm×40 cm, and the resultant sample was left at rest in an environment of 23°C±2°C under no load for 24 hours. Then, measurement was performed according to the method E of ISO 2439 (2008) by using AUTOGRAPH AG-X plus manufactured by Shimadzu Corporation in an environment of 23°C±2°C. Specifically, a pressure application plate having a diameter (φ) of 200 mm was disposed at the center position of the sample, and a thickness thereof at which the load became 5 N was measured. This thickness was regarded as an initial hardness tester thickness. With the position of the pressure application plate at this time being defined as a zero point, preliminary compression by 75% of the initial hardness tester thickness was performed at a speed of 100 mm/min one time, and the pressure application plate was returned to the zero point at the same speed. Then, the sample was left at rest for 4 minutes in this state. Immediately thereafter, compression by 25%, 40%, and 65% of the initial hardness tester thickness was performed (compression was performed so as to obtain thicknesses that were 75%, 60%, and 35% of the initial hardness tester thickness) at a speed of 100 mm/min, and the loads (unit: N/φ200) at this time were measured. These loads were respectively regarded as a 25%-compression hardness, a 40%-compression hardness, and a 65%-compression hardness (average values with n=3 being satisfied).

In addition, a value resulting from dividing the 65%-compression hardness by the 25%-compression hardness was regarded as a compressive deflection coefficient. The aforementioned operation was performed three times, and an average value (n=3) of the compressive deflection coefficients was obtained.

### (10) Residual Strain after 750-N Constant Load Repeated Compression

Each of the three-dimensional network structures was cut into a size of 40 cm×40 cm, and an initial hardness tester thickness (e) thereof was measured through the method described in the above (9). Thereafter, the sample, the thickness of which had been measured, was subjected to 750-N constant load repeated compression according to the method A (constant load method) of JIS K 6400-4 (2004) by using ASKER STM-536 manufactured by KOBUNSHI KEIKI CO., LTD. As a pressure applicator, a circular flat-lower-surface pressure applicator that had a bottom surface with an edge portion having a curvature radius of 25±1 mm and that had a diameter of 250±1 mm was used. The load was set to 750 N±20 N, the frequency of the compression was set to 70±5 times per minute, the number of times of the compression was set to 80,000 times, and the time during which the applied pressure was kept at the maximum of 750±20 N was set to 25% or less of the time required for the repeated compression. After the repeated compression was ended, the sample was left at rest for 10±0.5 minutes in a state where no force was applied. Using AUTOGRAPH AG-X plus manufactured by Shimadzu Corporation, the sample was disposed such that a pressure application plate having a diameter (φ) of 200 mm was located at the center position of the sample, and a thickness thereof at which the load became 5 N was measured. This thickness was regarded as a post-repeated-compression hardness tester thickness (f). The values of the initial hardness tester thickness (e) and the post-repeated-compression hardness tester thickness (f) were inputted to the following formula to obtain a residual strain after 750-N constant load repeated compression. The aforementioned operation was performed three times, residual strains after 750-N constant load repeated compression were calculated at the respective times of operation, and an average value (n=3) of the residual strains was regarded as a residual strain after 750-N constant load repeated compression of this sample. Residual strain after 750-N constant load repeated compression (unit: %)={(e)-(f)/(e)}×100

### (11) 40%-Compression Hardness Retention Rate after 750-N Constant Load Repeated Compression

Each of the samples was cut into a size of 40 cm×40 cm, and an initial hardness tester thickness and a 40%-compression hardness (g) thereof were measured through the method described in the above (9). Thereafter, the sample subjected to the measurement was subjected to 750-N constant load repeated compression according to the method A (constant load method) of JIS K 6400-4 (2004) by using ASKER STM-536 manufactured by KOBUNSHI KEIKI CO., LTD. As a pressure applicator, a circular flat-lower-surface pressure applicator that had a bottom surface with an edge portion having a curvature radius of 25±1 mm and that had a diameter of 250±1 mm was used. The load was set to 750 N±20 N, the frequency of the compression was set to 70±5 times per minute, the number of times of the compression was set to 80,000 times, and the time during which the applied pressure was kept at the maximum of 750±20 N was set to 25% or less of the time required for the repeated compression. After the repeated compression was ended, the sample was left at rest for 10±0.5 minutes in a state where no force was applied. Using AUTOGRAPH AG-X plus manufactured by Shimadzu Corporation, the sample was disposed such that a pressure application plate having a diameter (φ) of 200 mm was located at the center position of the sample, and the thickness of the sample was obtained as follows. That is, with the initial hardness tester thickness before 750-N constant load repeated compression being defined as a zero point, preliminary compression by 75% of the initial hardness tester thickness was performed at a speed of 100 mm/min one time, and the pressure application plate was returned to the zero point at the same speed. Then, the sample was left at rest for 4 minutes in this state. Immediately thereafter, compression by 40% of the initial hardness tester thickness was performed at a speed of 100 mm/min. The load at this time was regarded as a 40%-compression hardness after 750-N constant load repeated compression (h). The value of the 40%-compression hardness after 750-N constant load repeated compression (h) was divided by the value of the 40%-compression hardness (g) to obtain a 40%-compression hardness retention rate after 750-N constant load repeated compression. The aforementioned operation was performed three times, 40%-compression hardness retention rates after 750-N constant load repeated compression were calculated at the respective times of operation, and an average value (n=3) of the compression hardness retention rates was regarded as a 40%-compression hardness retention rate after 750-N constant load repeated compression of this sample.

### (12) 65%-Compression Hardness Retention Rate after 750-N Constant Load Repeated Compression

Each of the three-dimensional network structures was cut into a size of 40 cm×40 cm, and an initial hardness tester thickness and a 65%-compression hardness (i) thereof were measured through the method described in the above (9). Thereafter, the sample subjected to the measurement was subjected to 750-N constant load repeated compression according to the method A (constant load method) of JIS K 6400-4 (2004) by using ASKER STM-536 manufactured by KOBUNSHI KEIKI CO., LTD. As a pressure applicator, a circular flat-lower-surface pressure applicator that had a bottom surface with an edge portion having a curvature radius of 25±1 mm and that had a diameter of 250±1 mm was used. The load was set to 750 N±20 N, the frequency of the compression was set to 70±5 times per minute, the number of times of the compression was set to 80,000 times, and the time during which the applied pressure was kept at the maximum of 750±20 N was set to 25% or less of the time required for the repeated compression. After the repeated compression was ended, the sample was left at rest for 10±0.5 minutes in a state where no force was applied. Using AUTOGRAPH AG-X plus manufactured by Shimadzu Corporation, the sample was disposed such that a pressure application plate having a diameter (φ) of 200 mm was located at the center position of the sample, and the thickness of the sample was obtained as follows. That is, with the initial hardness tester thickness before 750-N constant load repeated compression being defined as a zero point, preliminary compression by 75% of the initial hardness tester thickness was performed at a speed of 100 mm/min one time, and the pressure application plate was returned to the zero point at the same speed. Then, the sample was left at rest for 4 minutes in this state. Immediately thereafter, compression by 65% of the initial hardness tester thickness was performed at a speed of 100 mm/min. The load at this time was regarded as a 65%-compression hardness after 750-N constant load repeated compression (j). The value of the 65%-compression hardness after 750-N constant load repeated compression (j) was divided by the value of the 65%-compression hardness (i) to obtain a 65%-compression hardness retention rate after 750-N constant load repeated compression. The aforementioned operation was performed three times, 65%-compression hardness retention rates after 750-N constant load repeated compression were calculated at the respective times of operation, and an average value (n=3) of the compression hardness retention rates was regarded as a 65%-compression hardness retention rate after 750-N constant load repeated compression of this sample.

The polybutylene adipate terephthalate resins were synthesized through the following methods.

### <Resin A>

In a reaction tank equipped with a stirrer, a thermometer, and a distillation cooler, 1,4-butanediol, adipic acid, and dimethyl terephthalate were mixed in proportions of 1.5 moles, 0.4 moles, and 0.6 moles, respectively. Then, the resultant mixture was fed with 300 ppm of tetrabutyl titanate (manufactured by Sigma-Aldrich Co., LLC.) as a titanium-based catalyst. Thereafter, a transesterification reaction and an esterification reaction were performed for 2 hours under a normal pressure and at 220°C, to prepare a prepolymer. The prepolymer was heated to 240°C, and then subjected to a polycondensation reaction at 0.1 mmHg for 2 hours. The obtained resin A was cooled, and then cut by using a pellet cutter, to produce pellets.

### <Resin B>

A resin B was produced in the same method as that for the resin A except that, unlike in the production of the resin A, the amounts of the adipic acid and the dimethyl terephthalate were changed to 0.53 moles and 0.47 moles, respectively. The obtained resin B was cooled, and then cut by using a pellet cutter, to produce pellets.

### <Resin C>

A resin C was produced in the same method as that for the resin A except that, unlike in the production of the resin A, the amounts of the adipic acid and the dimethyl terephthalate were changed to 0.50 moles and 0.50 moles, respectively. The obtained resin C was cooled, and then cut by using a pellet cutter, to produce pellets.

### [Example 1]

Pellets of the obtained resin A were extruded from a nozzle at a spinning temperature of 240°C downward of the nozzle at a single-hole extrusion rate of 1.0 g/min. The nozzle had a nozzle effective surface measuring 680 mm in a width direction and having a width of 64 mm in a thickness direction. In the nozzle effective surface, orifices each having a hole diameter of 1.0 mm were arranged in a staggered manner at an inter-hole pitch of 5 mm. The ambient temperature was set to 30°C, and cooling air having a temperature of 80°C was applied at a speed of 0.1 m per second over a range of 10 to 20 cm immediately below the nozzle from one surface in the thickness direction of the extruded filament in a molten state. Cooling water was located 30 cm below the nozzle surface, and a pair of take-up conveyors were disposed to be partially exposed to above the surface of the water such that endless nets thereof made of stainless steel were parallel, with an opening width of 48 mm as a gap. With this, the extruded filament in a molten state was curved and twisted to form a loop and fuse contact portions, and accordingly, a network configuration was formed. While both surfaces of the resultant network body in a molten state were sandwiched by the take-up conveyors, the network body was drawn into the cooling water at a speed of 0.75 m per minute and was solidified to flatten both surfaces. Then, the network body was cut into a predetermined size and was subjected to drying heat treatment for 20 minutes with hot air at 90°C. Consequently, a three-dimensional network structure was obtained. The obtained three-dimensional network structure was a three-dimensional network structure that satisfied the requirements of the present invention and that had excellent repeated compression durability.

### [Example 2]

A three-dimensional network structure was obtained in the same manner as in Example 1, except that: a nozzle having orifices that were arranged in a staggered manner at an inter-hole pitch of 8 mm and that each had a triple-bridge hollow-forming cross section with an outer diameter of 5.0 mm and an inner diameter of 4.4 mm was used; the single-hole extrusion rate was set to 3.9 g/min; the take-up speed was set to 2.26 m/min without applying cooling air by passage through a cooling space at an ambient temperature of 40°C; and the distance between the nozzle surface and the cooling water was set to 39 cm. The obtained three-dimensional network structure was a three-dimensional network structure that satisfied the requirements of the present invention and that had excellent repeated compression durability.

### [Example 3]

A three-dimensional network structure was obtained in the same manner as in Example 2, except that: a product obtained by adding 0.06% by mass of water with respect to 100% by mass of a solid component of the resin A as a raw material was used instead of pellets of the resin A; the spinning temperature was set to 230°C; the ambient temperature was set to 30°C; the cooling air temperature was set to 100°C; the cooling air speed was set to 0.3 m per second; the take-up speed was set to 2.14 m/min; and the distance between the nozzle surface and the cooling water was set to 34 cm. The obtained three-dimensional network structure was a three-dimensional network structure that satisfied the requirements of the present invention and that had excellent repeated compression durability.

### [Example 4]

A three-dimensional network structure was obtained in the same manner as in Example 2, except that: the spinning temperature was set to 230°C; the ambient temperature was set to 30°C; the cooling air temperature was set to 100°C; the cooling air speed was set to 0.3 m per second; the take-up speed was set to 2.00 m/min; and the distance between the nozzle surface and the cooling water was set to 42 cm. The obtained three-dimensional network structure was a three-dimensional network structure that satisfied the requirements of the present invention and that had excellent repeated compression durability.

### [Example 5]

A three-dimensional network structure was obtained in the same manner as in Example 4, except that: pellets of the resin C were used instead of pellets of the resin A; the single-hole extrusion rate was set to 3.3 g/min; the cooling air speed was set to 0.1 m per second; the take-up speed was set to 1.70/min; and the distance between the nozzle surface and the cooling water was set to 37 cm. The obtained three-dimensional network structure was a three-dimensional network structure that satisfied the requirements of the present invention and that had excellent repeated compression durability.

### [Comparative Example 1]

A three-dimensional network structure was obtained in the same manner as in Example 2, except that: the spinning temperature was set to 220°C; the ambient temperature was set to 30°C; the take-up speed was set to 1.86 m/min without applying cooling air; and the distance between the nozzle surface and the cooling water was set to 44 cm. The obtained three-dimensional network structure was a three-dimensional network structure that did not satisfy the requirements of the present invention and that was inferior in repeated compression durability.

### [Comparative Example 2]

A three-dimensional network structure was obtained in the same manner as in Example 2, except that: pellets of the resin B were used instead of pellets of the resin A; the spinning temperature was set to 190°C; the single-hole extrusion rate was set to 2.5 g/min; the ambient temperature was set to 20°C; the take-up speed was set to 1.62/min without applying cooling air; the distance between the nozzle surface and the cooling water was set to 35 cm; and the temperature in the hot air drying was set to 80°C. The obtained three-dimensional network structure was a three-dimensional network structure that did not satisfy the requirements of the present invention and that was inferior in repeated compression durability.

Table 1 shows production conditions and the characteristics of the obtained three-dimensional network structure in Examples from 1 to 5 and Comparative Examples from 1 to 2. In Table 1, the characteristic value is the average of the value by operations of multiple times.

**[Table 1]**

| | | Example 1 | Example 2 | Example 3 | Example 4 | Example 5 | Comparative Example 1 | Comparative Example 2 |
|---|---|---|---|---|---|---|---|---|
| Manufacturing conditions | Spinning temperature: °C | 240 | 240 | 230 | 230 | 230 | 220 | 190 |
| | Single-hole extrusion rate: g/min | 1.0 | 3.9 | 3.9 | 3.9 | 3.3 | 3.9 | 2.5 |
| | Ambient temperature: °C | 30 | 40 | 30 | 30 | 30 | 30 | 20 |
| | Cooling air temperature: °C | 80 | - | 100 | 100 | 100 | - | - |
| | Cooling air speed: m/sec | 0.1 | 0 | 0.3 | 0.3 | 0.1 | 0 | 0 |
| | Distance (from nozzle surface to surface of cooling water in water tank): cm | 30 | 39 | 34 | 42 | 37 | 44 | 35 |
| | Take-up speed: m/min | 0.75 | 2.26 | 2.14 | 2.00 | 1.70 | 1.86 | 1.62 |
| Resin | Resin | A | A | A | A | C | A | B |
| | PBAT content: % by mass | 100 | 100 | 100 | 100 | 100 | 100 | 100 |
| | Molar ratio (terephthalic acid residue/adipic acid residue) | 1.5 | 1.5 | 1.5 | 1.5 | 1 | 1.5 | 0.89 |
| | Resin melting point: °C | 150 | 150 | 150 | 150 | 130 | 150 | 120 |
| | Melt flow rate: g/10 min | 6.5 | 6.5 | 10.6 | 6.5 | 11 | 6.5 | 20 |
| Three-dimensional network structure | Average fiber diameter of surface layer portion: mm | 0.58 | 0.88 | 0.92 | 0.87 | 0.89 | 0.81 | 0.81 |
| | Average fiber diameter of inner layer portion: mm | 0.52 | 0.80 | 0.81 | 0.78 | 0.81 | 0.78 | 0.79 |
| | Average fiber diameter of surface layer portion/average fiber diameter of inner layer portion: times | 1.12 | 1.10 | 1.14 | 1.12 | 1.10 | 1.04 | 1.03 |
| | Average fiber diameter of continuous filament: mm | 0.55 | 0.84 | 0.87 | 0.83 | 0.85 | 0.80 | 0.80 |
| | Melting-start onset temperature: °C | 115.2 | 117.6 | 101.7 | 110.8 | 96.0 | 117.1 | 93.8 |
| | Enthalpy of fusion: J/g | 24.0 | 25.6 | 23.4 | 25.0 | 24.0 | 24.9 | 18.7 |
| | Low-temperature phase onset temperature: °C | 34.6 | 40.4 | 43.9 | 38.8 | 36.2 | 36.8 | 38.2 |
| | Low-temperature phase enthalpy: J/g | 1.40 | 1.00 | 0.52 | 0.71 | 1.50 | 1.18 | 2.90 |
| | Apparent density: g/cm³ | 0.041 | 0.038 | 0.036 | 0.040 | 0.041 | 0.043 | 0.042 |
| | Thickness: mm | 37.1 | 47.4 | 50.9 | 50.7 | 50.1 | 50.4 | 38.7 |
| | 40°C-compression residual strain: % | 13.2 | 15.0 | 12.8 | 14.9 | 16.2 | 16.3 | 18.6 |
| | 25%-compression hardness: N/Φ200 | 56 | 126 | 117 | 132 | 104 | 139 | 94 |
| | 40%-compression hardness: N/Φ200 | 93 | 163 | 153 | 220 | 159 | 223 | 151 |
| | 65%-compression hardness: N/Φ200 | 166 | 365 | 320 | 493 | 332 | 338 | 230 |
| | Residual strain after 750-N constant load repeated compression: % | 9.5 | 8.2 | 9.8 | 9.9 | 9.7 | 11.1 | 9.9 |
| | 40%-compression hardness retention rate after 750-N constant load repeated compression: % | 49.6 | 56.2 | 50.0 | 50.0 | 48.5 | 43.8 | 41.8 |
| | 65%-compression hardness retention rate after 750-N constant load repeated compression: % | 62.7 | 68.0 | 63.2 | 62.8 | 62.2 | 55.3 | 60.1 |
| | Compressive deflection coefficient | 3.0 | 2.9 | 2.7 | 3.7 | 3.2 | 2.4 | 2.4 |

## Claims

1. A three-dimensional network structure having a three-dimensional random loop-bonded configuration and comprising a continuous filament made from a thermoplastic resin composition, wherein
the thermoplastic resin composition contains 70% by mass or more of a polybutylene adipate terephthalate resin,
an enthalpy of an endothermic peak, in which a differential scanning calorimetry curve regarding the continuous filament measured by using a differential scanning calorimeter has a minimum value in a range from 30°C to 70°C, is 2.5 J/g or less,
the continuous filament has an average fiber diameter of 0.1 mm or more and 3.0 mm or less,
an average fiber diameter of a surface layer portion of the three-dimensional network structure is not less than 1.05 times an average fiber diameter of an inner layer portion of the three-dimensional network structure, and
the three-dimensional network structure has an apparent density of 0.01 g/cm³ or more and 0.20 g/cm³ or less, a residual strain after 750-N constant load repeated compression of 15% or less, and a 40%-compression hardness retention rate after 750-N constant load repeated compression of 45% or more.

2. The three-dimensional network structure according to claim 1, wherein
the polybutylene adipate terephthalate resin contains an adipic acid residue and a terephthalic acid residue, and
a molar ratio of the terephthalic acid residue to the adipic acid residue is 1.0 or more and 3.0 or less.

3. The three-dimensional network structure according to claim 1 or 2, wherein the polybutylene adipate terephthalate resin has a melting point of 125°C or more and 180°C or less.

4. The three-dimensional network structure according to claim 1 or 2, wherein the three-dimensional network structure has a 65%-compression hardness retention rate after 750-N constant load repeated compression of 60% or more.

5. The three-dimensional network structure according to claim 1 or 2, wherein the three-dimensional network structure has a compressive deflection coefficient of 2.5 or more.

6. The three-dimensional network structure according to claim 1 or 2, wherein the three-dimensional network structure has a thickness of 10 mm or more and 300 mm or less.

7. The three-dimensional network structure according to claim 1 or 2, wherein the three-dimensional network structure has a 40°C-compression residual strain of 25% or less.
